

## UNITED STATES PATENT OFFICE

2,552,570

## OXIDATION RESISTING HYDROCARBON PRODUCTS

John G. McNab, Cranford, Nilo V. Hakala, Rahway, and John P. McDermott, Roselle, N. J., assignors to Standard Oil Development Company, a corporation of Delaware

No Drawing. Application November 28, 1947,  
Serial No. 788,670

3 Claims. (Cl. 252—32.7)

1

The present invention relates to the improvement of hydrocarbon products and in particular to the improvement of mineral lubricating oil compositions by the incorporation therein of a class of additives which impart oxidation resisting properties to such products.

In the development of petroleum lubricating oils the trend has been to use more and more efficient refining methods in order to reduce the tendency of the oils to form carbon and deposits of solid matter or sludge. While such highly refined oils possess many advantages, their resistance to oxidation particularly under conditions of severe service is generally decreased and they are more prone to form soluble acidic oxidation products which are corrosive. They are generally less effective than the untreated oils in protecting the metal surfaces which they contact against rusting and corrosion due to oxygen and moisture. They also often deposit thick films of "varnish" on hot metal surfaces, such as the pistons of internal combustion engines.

In accordance with the present invention a new class of compounds has been discovered, which when added to refined mineral lubricating oils and other hydrocarbon products in small portions substantially reduce the tendency of such products to corrode metal surfaces, particularly the surfaces of copper-lead and cadmium-silver bearings which are employed in internal combustion engines, and they are effective generally for the purpose of inhibiting oxidation of hydrocarbon products which are exposed to the action of atmospheric oxygen. It is well known that many compounds of copper, especially certain organic salts such as copper naphthenate, as well as metallic copper, tend to promote the oxidation of organic material such as hydrocarbons. Most, if not all, of the copper compounds having this property are cupric, that is, higher valent compounds. However, it has been found in accordance with the present invention that certain cuprous salts, more specifically the cuprous salts of organo-thiophosphoric acids, have the property of inhibiting the oxidation of hydrocarbons to a marked degree.

The class of compounds comprising the antioxidant additives of the present invention are more accurately defined as the compounds having the general formula



where R and R' are hydrocarbon radicals, more

2

specifically alkyl, alkenyl, cycloaliphatic, alkaryl, or aralkyl radicals, and in general any radicals, whether aliphatic or aromatic, which contain a total of at least 10 carbon atoms in the combined aliphatic groups, whether or not attached to aromatic nuclei. In this specification and the appended claims the term "aliphatic" is intended to include both open chain and closed chain groups, saturated or unsaturated, straight chain or branched. The invention also includes compounds of the above type which contain substituted halogen atoms or nitro groups. Compounds of the aliphatic radical type, that is, those having no aromatic nuclei, are generally preferred. In the above general formula X represents oxygen or sulfur.

The cuprous salts of the class described above may be readily prepared by treating an organo-thiophosphoric acid with cuprous oxide, preferably in the presence of a small amount of a reducing agent, such as sodium hydrosulfite, which appears to give a product of lighter color and free from copper staining characteristics. The organo-thiophosphoric acid may be prepared by known means, such as by reacting a suitable alcohol with phosphorus pentasulfide:

The preparation of the thiophosphoric acid and its conversion to the cuprous salt may be illustrated by the following equations in which R represents the organic radical of the original alcohol or phenol:



Instead of using a single alcohol, it is entirely feasible to prepare an organo-thiophosphoric acid by treating a mixture of two or more alcohols with phosphorus pentasulfide and to prepare a cuprous salt useful in accordance with the present invention by neutralizing the acid product of such a reaction with cuprous oxide. The exact constitution of the acid prepared from a mixture of alcohols is not known, although it is believed that the product consists largely of a mixed organo-thiophosphoric acid containing two different organic radicals. By employing mixtures of alcohols it is possible to make use of a certain proportion of short chain alcohols, since it is only necessary that the total number

of the carbon atoms in the organic radicals be as great as 10 in order to give the product sufficient solubility in the hydrocarbon base stock.

Instead of alcohols or phenols, mercaptans or thiophenols may be employed in the original preparation of the thiophosphoric acid. Acids prepared by the reaction of phosphorus pentasulfide with mercaptans or thiophenols will have sulfur atoms linking the phosphorus atoms with the organic groups.

Among the alcohols which are generally preferred for use as starting materials in the preparation of the salts of the present invention may be mentioned 2-ethylhexanol, methylcyclohexanol, a commercial mixture of C<sub>12</sub> to C<sub>16</sub> alcohols, alcohols prepared by the reaction of an olefin with carbon monoxide and hydrogen and subsequent hydrogenation of the product so formed, such as octyl alcohol and nonyl alcohol formed in this manner, and other products of similar composition and derivation. The above are specifically mentioned because of their commercial availability, but other alcohols falling within the general class described may be employed, such as the normal straight-chain alcohols, alcohols derived from natural waxes, alcohols produced by the oxidation of petroleum hydrocarbon products, lauryl alcohol, stearyl alcohol, oleyl alcohol, naturally occurring alcohols such as those found in wool fat, sperm oil, and the like. As discussed above, mixtures of alcohols may be employed as well as single alcohols. A mixture of isopropanol and 2-ethylhexanol is particularly satisfactory.

For the preparation of thiophosphoric acids containing alkaryl groups, alkylated phenols, alkylated naphthols, and the like may be employed in the place of alcohols, and the method is analogous. Preferred examples of alkylated phenols are amyl phenols, octyl phenols, wax-alkylated phenols, petroleum phenols, and like products, including mixtures of phenols.

For general antioxidant purposes and particularly when the additives are to be employed in mineral lubricating oils, the amount of the additives will range from about 0.02% to about 3%, and the particular amount in individual cases will be selected in accordance with the requirements of the case and in view of the properties of the base stock employed. Since cuprous organothiophosphates prepared from C<sub>8</sub> alcohols or higher are completely miscible with lubricating oil, it is convenient for commercial purposes to prepare concentrates containing from 25 to 75% by weight of the additive in mineral lubricating oil, and to transport and blend the additives in the form of such concentrates. Concentrates containing about 40% of the additive are very conveniently prepared.

The preparation and testing of samples of the additives of the present invention as well as samples of analogous salts of other metals for comparison are illustrated by the examples to be described in detail below, but such examples are not to be construed as limiting the scope of the invention in any manner.

*Example 1.—Preparation of cuprous 2-ethylhexyl thiophosphate*

A mixture of 520.8 g. (4 mols) of 2-ethylhexanol and 222 g. (1 mol) of P<sub>2</sub>S<sub>5</sub> was heated for 1½ hours at 90° C. in a 3-necked, 2-liter flask equipped with a stirrer, reflux condenser and thermometer. The product was then filtered to remove a small amount of insoluble material.

70  
75

The thiophosphoric acid was then added dropwise, with stirring, to a slurry of 143 g. (1 mol) of Cu<sub>2</sub>O and 17.4 g. of sodium hydrosulfite in 600 cc. of benzene over a period of 3½ hours (maximum temperature 40° C.). After stirring for an additional hour, the product was filtered. The clear dark brown filtrate was mixed with enough of a light SAE 10 grade mineral oil to give as a final product a 40% concentrate. This solution was then placed on a steam bath with nitrogen blowing for 24 hours to remove the benzene and water. Upon analysis, this concentrate was found to contain 5.8% copper and 5.7% sulfur; theoretical values were 6.1% copper and 6.1% sulfur.

*Example 2.—Preparation of cuprous nonyl thiophosphate*

This preparation was carried out in the same manner as that described in Example 1, using 576 g. of nonyl alcohol (a branched chain C<sub>9</sub> alcohol prepared by reacting diisobutylene, carbon monoxide and hydrogen and hydrogenating the product), 222 g. of P<sub>2</sub>S<sub>5</sub>, 143 g. of Cu<sub>2</sub>O, and 17.4 g. of sodium hydrosulfite.

Upon analysis, the 40% oil concentrate was found to contain 6.3% copper and 7.0% sulfur; theoretical values were 6.3% copper and 6.4% sulfur.

*Example 3.—Preparation of cuprous octyl thiophosphate*

A mixture of 520 g. (4 mols) of octyl alcohol (a branched chain C<sub>8</sub> alcohol prepared by reacting a C<sub>7</sub> olefin polymer, carbon monoxide and hydrogen and hydrogenating the product), and 222 g. (1 mol) of P<sub>2</sub>S<sub>5</sub> was heated for 1½ hours at 90° C., in a 3-necked, 2-liter flask equipped with a stirrer, reflux condenser, and thermometer. The thiophosphoric acid was then poured into a 4-liter beaker containing 1126 g. of diluent oil (a light lubricating oil of approximately SAE 10 grade). With rapid stirring and nitrogen blowing, a mixture of 17.4 g. of sodium hydrosulfite and 128.7 g. of Cu<sub>2</sub>O was added in small portions over a period of about 50 minutes, during which time the temperature rose from 40° C. to 55° C. After stirring for an additional 1.5 hours at 105° C., the product was filtered. A clear, dark brown concentrate was obtained, which upon analysis was found to contain 5.6% copper, 3.1% phosphorus and 6.5% sulfur.

*Example 4.—Preparation of cuprous methylcyclohexyl thiophosphate*

A 3-necked, 1-liter flask, equipped with a stirrer, reflux condenser and thermometer, was charged with 228 g. (2 mols) of methylcyclohexanol and 111 g. (½ mol) of P<sub>2</sub>S<sub>5</sub>. This mixture was heated with stirring at 110° C., for 30 minutes, after which the resulting thiophosphoric acid was poured into a 3-liter beaker containing 514 g. of a light lubricating oil of approximately SAE 10 grade. This solution was then heated to 50° C., after which 71.5 g. (½ mol) of Cu<sub>2</sub>O was added in small portions over a period of 30 minutes with rapid stirring and nitrogen blowing (temperature rose to 90° C.). After stirring for an additional twenty minutes at 110° C., the product was filtered, a clear, dark red, viscous concentrate being obtained. Upon analysis it was found to contain 7.3% copper, 7.1% sulfur, and 3.4% phosphorus.

**Example 5.—Preparation of cuprous isopropyl ethylhexyl thiophosphate**

The isopropyl-ethylhexyl thiophosphoric acid mixture was prepared as described in Example 1, using a mixture of 90 g. (1.5 mol) of isopropanol and 130 g. (1 mol) of ethylhexanol. The acid mixture was poured into 561 g. of a light lubricating oil of approximately SAE 10 grade, and after heating to 50° C., 88.7 g. of Cu<sub>2</sub>O was added in small portions over a period of about 30 minutes. After stirring for an additional 2 hours at 105° C., with nitrogen blowing, the product was filtered, a clear, deep red concentrate being obtained, which upon analysis was found to contain 7.3% copper, 7.4% sulfur, and 3.7% phosphorus, indicating the product to be a 40% oil concentrate containing cuprous isopropyl thiophosphate, cuprous ethylhexyl thiophosphate and/or the cuprous salt of mixed isopropyl-ethylhexyl thiophosphoric acid. This concentrate remained clear after standing for 2 weeks at 30° F.

**Example 6.—Preparation of cuprous C<sub>12</sub>—C<sub>16</sub> alkyl-secondary butyl thiophosphate**

This preparation was carried out in the same manner as that described in Example 5, using a mixture of 104 g. of a commercial mixture of C<sub>12</sub>—C<sub>16</sub> alcohol and 207 g. of secondary butyl alcohol, 184 g. of P<sub>2</sub>S<sub>5</sub>, 74.4 g. Cu<sub>2</sub>O, and 768 g. of the same diluent oil as used in Example 5. The final product was found to contain 7.3% copper, 7.5% sulfur and 3.6% phosphorus, indicating it to be a 40% oil concentrate containing cuprous secondary butyl thiophosphate, cuprous C<sub>12</sub>—C<sub>16</sub> alkyl thiophosphate and/or the cuprous salt of mixed secondary butyl-C<sub>12</sub>—C<sub>16</sub> alkyl thiophosphoric acid. This concentrate remained clear after storage for 2 weeks at 30° F.

**Example 7.—Preparation of calcium ethylhexyl thiophosphate**

The ethylhexyl thiophosphoric acid was prepared as described in Example 1. The calcium salt was then prepared in the same manner as described in Example 5, using CaO as the neutralizing agent.

**Example 8.—Preparation of potassium ethylhexyl thiophosphate**

This preparation was carried out in the same manner as that described in Example 7, using KOH as the neutralizing agent. Upon cooling this concentrate to room temperature, a considerable amount of the potassium salt precipitated out of solution.

**Example 9.—Preparation of sodium ethylhexyl thiophosphate**

This preparation was carried out in the same manner as that described in Example 7, using NaOH as the neutralizing agent.

**Example 10.—Preparation of zinc ethylhexyl thiophosphate**

This preparation was carried out in the same manner as that described in Example 7, using ZnO as the neutralizing agent.

**Example 11.—Laboratory bearing corrosion tests**

Blends containing 0.25% each of various cuprous salts prepared as described in preceding examples in an extracted Mid-Continent lubricating oil of paraffinic SAE 20 grade and a sample of the unblended base oil were submitted to a laboratory test designed to measure the

effectiveness of the new additives in inhibiting the corrosiveness of a typical mineral lubricating oil toward the surfaces of copper-lead bearings. The test was conducted as follows:

- 5 500 cc. of the oil was placed in a glass oxidation tube (13 inches long and 2½ inches in diameter) fitted at the bottom with a ¼ inch air inlet tube perforated to facilitate air distribution. The oxidation tube was then immersed in a heating bath so that the oil temperature was maintained at 325° F. during the test. Two quarter sections of automotive bearings of copper-lead alloy of known weight having a total area of 25 sq. cm. were attached to opposite sides of a stainless 10 steel rod which was then immersed in the test oil and rotated at 600 R. P. M., thus providing sufficient agitation of the sample during the test. Air was then blown through the oil at the rate of 2 cu. ft. per hour. At the end of each 4-hour 15 period the bearings were removed, washed with naphtha and weighed to determine the amount of loss by corrosion. The bearings were then repolished (to increase the severity of the test), reweighed, and then subjected to the test for 20 additional 4-hour periods in like manner. The results are given in the following table as "corrosion life," which indicates the number of hours required for the bearings to lose 100 mg. in weight, determined by interpolation of the data 25 obtained in the various periods.

|    | Oil Blend                                                                                           | Bearing Corrosion Life, Hrs. |
|----|-----------------------------------------------------------------------------------------------------|------------------------------|
| 35 | Base Oil                                                                                            | 9                            |
|    | Base oil+0.25% cuprous ethylhexyl thiophosphate (Ex. 1)                                             | 22                           |
|    | Base oil+0.25% cuprous nonyl thiophosphate (Ex. 2)                                                  | 21                           |
|    | Base oil+0.25% cuprous octyl thiophosphate (Ex. 3)                                                  | 18                           |
|    | Base oil+0.25% cuprous methylcyclohexyl thiophosphate (Ex. 4)                                       | 27                           |
| 40 | Base oil+0.25% cuprous isopropylethylhexyl thiophosphate (Ex. 5)                                    | 26                           |
|    | Base oil+0.25% cuprous C <sub>12</sub> —C <sub>16</sub> alkyl-secondary butyl thiophosphate (Ex. 6) | 33                           |

**Example 12.—Lauson engine tests**

Blends containing 0.6% each of various products prepared as described in the foregoing examples in a solvent extracted Mid-Continent paraffinic lubricating oil of SAE 10 grade and a sample of the unblended base oil were employed as crankcase lubricants in tests with a Lauson engine operating at 300° F. jacket temperature, 295° F. oil temperature, 1800 R. P. M. speed, and 1.5 indicated kilowatt load, the tests being conducted for 20 hours each. The loss in weight of the copper-lead bearing and the varnish demerit were determined in each test. The varnish demerit rating was based upon a method of rating in which a perfectly clean piston surface is given a rating of 0 and a demerit of 10 is given to the worst condition which could be expected to exist of that surface. The results of these observations are as follows:

|    | Base Oil                                                 | Varnish Demerit | Bearing Weight Loss (Mg./ Bearing) |
|----|----------------------------------------------------------|-----------------|------------------------------------|
| 65 | Base oil                                                 | 3.5             | 220                                |
|    | Base oil+0.6% cuprous ethylhexyl thiophosphate (Ex. 1)   | 1.5             | 20                                 |
| 70 | Base oil+0.6% calcium ethylhexyl thiophosphate (Ex. 7)   | 2.8             | 37                                 |
|    | Base oil+0.6% potassium ethylhexyl thiophosphate (Ex. 8) | 4.3             | 19                                 |
|    | Base oil+0.6% sodium ethylhexyl thiophosphate (Ex. 9)    | 6.0             | 32                                 |

*Example 13.—Chevrolet engine tests*

Blends containing products of various preceding examples in a solvent extracted Mid-Continent paraffinic SAE 10 oil in the amounts indicated below and a sample of the unblended base oil were employed as the crankcase oil in 36-hour tests with a Chevrolet engine operated at 30 brake H. P., 3150 R. P. M. speed, 280° F. oil temperature and 200° F. jacket temperature. After each test was completed, the weight loss of the copper-lead bearing was determined. The results are shown in the following table:

| Oil Blend                                                       | Bearing Weight Loss (Gm./ Bearing) |
|-----------------------------------------------------------------|------------------------------------|
| Base Oil                                                        | 8.91                               |
| Base oil+0.6% cuprous ethylhexyl thiophosphate (Ex. 1)          | 0.09                               |
| Base oil+0.3% cuprous ethylhexyl thiophosphate (Ex. 1)          | 0.15                               |
| Base oil+0.6% cuprous nonyl thiophosphate (Ex. 2)               | 0.11                               |
| Base oil+0.6% cuprous octyl thiophosphate (Ex. 3)               | 0.30                               |
| Base oil+0.6% cuprous isopropylethylhexyl thiophosphate (Ex. 5) | 0.05                               |

The above data indicate clearly that the additives of the present invention are very effective in reducing bearing corrosion as well as being somewhat effective in also reducing varnish formation on the piston surface. It may also be observed that the cuprous salts are generally more effective than the alkali metal salts. Although the potassium ethylhexyl thiophosphate reduced the bearing corrosion to the same extent as the corresponding cuprous salt in the Lauson engine test, it will be observed that the potassium salt caused a greater amount of varnish formation than the unblended base oil, while the cuprous salt reduced the varnish formation.

The new additives of the present invention, while effective in inhibiting bearing corrosion, do not always inhibit the tendency of the oil to deposit varnish on engine parts to the desired extent, and it is accordingly advantageous to employ in combination with these additives other additives which have a detergent action. Among the most useful of such detergent additives are metal phenates, sulfurized metal phenates, sulfurized metal salts of phenol sulfides, reaction products of metal phenates and metal salts of phenol sulfide with sulfides of phosphorus, metal carboxylates, metal sulfonates, and the like. The following example illustrates the advantages realized in employing a combination of additives.

*Example 14.—Chevrolet engine tests of additive combinations in lubricating oil*

Blends were prepared containing cuprous ethylhexyl thiophosphate (prepared as in Example 1) alone and in combination with certain detergent additives as shown in the table below. Tests were also made of the base oil, which was a solvent extracted Mid-Continent paraffinic SAE 10 oil which was of a different lot and higher sulfur content from the oil employed in the tests of Example 13. Tests were also made with a blend of this oil with a typical detergent additive alone. The tests were conducted in the manner described in Example 13, while the varnish demerit ratings were made according to the system described in Example 12. The results of these tests are as follows:

| Oil Blend                                                                                                                             | Varnish Demerit | Cu-Pb Bearing Weight Loss (Gm./ Bearing) |
|---------------------------------------------------------------------------------------------------------------------------------------|-----------------|------------------------------------------|
| Base oil                                                                                                                              | 0.13            | 2.06                                     |
| Base oil+0.6% cuprous ethylhexyl thiophosphate                                                                                        | 3.79            | 0.09                                     |
| Base oil+0.7% barium tert.-octyl phenol sulfide—P <sub>2</sub> S <sub>5</sub> reaction product                                        | 0.35            | 0.65                                     |
| Base oil+0.18% cuprous ethylhexyl thiophosphate+0.7% barium tert.-octyl phenol sulfide—P <sub>2</sub> S <sub>5</sub> reaction product | 0.88            | 0.16                                     |
| Base oil+0.45% cuprous ethylhexyl thiophosphate+0.5% calcium petroleum sulfonate                                                      | 2.06            | 0.10                                     |

15 The above data show that extremely good results are obtained from the combination of the cuprous alkyl thiophosphate and the barium octyl phenol sulfide—P<sub>2</sub>S<sub>5</sub> reaction product, with regard to both varnish demerit and bearing corrosion.

20 The products of the present invention may be employed not only in ordinary hydrocarbon lubricating oils but also in the "heavy duty" type of lubricating oils which have been compounded

25 with such detergent type additives as metal soaps, metal petroleum sulfonates, metal phenates, metal alcoholates, metal alkyl phenol sulfides, metal organo phosphates, thiophosphates, phosphites and thiophosphites, metal salicylates, metal xanthates and thioxanthates, metal thiocarbamates, amines and amine derivatives, reaction products of metal phenates and sulfur, reaction products of metal phenates and phosphorus sulfides, metal phenol sulfonates and the like. Thus the additives

30 of the present invention may be used in lubricating oils containing such other addition agents as barium tert.-octylphenol sulfide, calcium tert.-amylphenol sulfide, nickel oleate, barium octadecylate, calcium phenyl stearate, zinc diisopropyl salicylate, aluminum naphthenate, calcium cetyl phosphate, barium di-tert.-amylphenol sulfide, calcium petroleum sulfonate, zinc methyl cyclohexyl thiophosphate, calcium di-chlorostearate, etc. Other types of additives,

35 such as phenols and phenol sulfides may be employed.

40 The lubricating oil base stocks used in the compositions of this invention may be straight mineral lubricating oils or distillates derived from paraffinic, naphthenic, asphaltic, or mixed base crudes, or, if desired, various blended oils may be employed as well as residuals, particularly those from which asphaltic constituents have been carefully removed. The oils may be refined by conventional methods using acid, 45 alkali and/or clay or other agents such as aluminum chloride, or they may be extracted oils produced, for example, by solvent extraction with solvents of the type of phenol, sulfur dioxide, furfural, dichlorodimethyl ether, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products.

50 In certain instances cracking coil tar fractions and coal tar or shale oil distillates may also be used. Also, for special applications, animal, vegetable or fish oils or their hydrogenated or volatilized products may be employed in admixture with mineral oils.

55 For the best results the base stock chosen should normally be that oil which without the new additive present gives the optimum performance in the service contemplated. However,

since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at 210° F. For the lubrication of certain low and medium speed Diesel engines the general practice has often been to use a lubricating oil base stock prepared from naphthenic or aromatic crudes and having a Saybolt viscosity at 210° F. of 45 to 90 seconds and a viscosity index of 0 to 50. However, in certain types of Diesel engine and other gasoline engine service, oils of higher viscosity index are often preferred, for example, up to 75 to 100, or even higher, viscosity index.

In addition to the material to be added according to the present invention, other agents may also be used such as dyes, pour depressors, heat thickened fatty oils, sulfurized fatty oils, organometallic compounds, metallic or other soaps, sludge dispersers, antioxidants, thickeners, viscosity index improvers, oiliness agent, resins, rubber olefinpolymers, voltolized fats, voltolized mineral oils, and/or voltolized waxes and colloidal solids such as graphite or zinc oxide, etc. Solvents and assisting agents, such as esters, ketones, alcohols, aldehydes, halogenated or nitrated compounds, and the like may also be employed.

Assisting agents which are particularly desirable as plasticizers and defoamers are the higher alcohols having eight or more carbon atoms and preferably 12 to 20 carbon atoms. The alcohols may be saturated straight and branched chain aliphatic alcohols such as octyl alcohol



lauryl alcohol ( $C_{12}H_{25}OH$ ), cetyl alcohol



stearyl alcohol, sometimes referred to as octadecyl alcohol, ( $C_{18}H_{37}OH$ ), heptadecyl alcohol ( $C_{17}H_{35}OH$ ), and the like; the corresponding olefinic alcohols such as oleyl alcohol; cyclic alcohols such as naphthenic alcohols; and aryl substituted alkyl alcohols, for instance, phenyl octyl alcohol, or octadecyl benzyl alcohol; or mixtures of these various alcohols, which may be pure or substantially pure synthetic alcohols. One may also use mixed naturally occurring alcohols such as those found in wool fat (which is known to contain a substantial percentage of

alcohols having about 16 to 18 carbon atoms) and in sperm oil (which contains a high percentage of cetyl alcohol); and although it is preferable to isolate the alcohols from those materials, for some purposes the wool fat, sperm oil or other natural products rich in alcohols may be used per se. Products prepared synthetically by chemical processes may also be used, such as alcohols prepared by the oxidation of petroleum hydrocarbons, e. g. paraffin wax, petrolatum, etc.

In addition to being employed in crankcase lubricants the additives of the present invention may also be used in extreme pressure lubricants, engine flushing oils, industrial oils, general machinery oils, process oils, rust preventive compositions and greases.

The additives of the present invention may be employed as antioxidant or stabilizing agents not only in mineral lubricating oils, but also in petroleum hydrocarbon products generally, where improved resistance to oxidation is desired. Thus the products may be added to motor oils, Diesel fuels, kerosene, waxes, hydrocarbon polymers, natural and synthetic rubbers, and the like.

The present invention is not to be considered as limited by any of the examples described herein, which are given by way of illustration only, but is to be limited solely by the terms of the appended claims.

We claim:

1. A composition consisting essentially of a hydrocarbon oil containing 0.02 to 3% of a compound of the approximate formula



where R and R' are  $C_8$  alkyl groups.

2. A composition according to claim 1 in which R and R' are 2-ethylhexyl groups.

3. A composition consisting essentially of a mineral lubricating oil, about 0.18% of cuprous 2-ethylhexyl thiophosphate, and about 0.7% of the reaction product of the barium salt of tert-octyl phenol sulfide and phosphorus pentasulfide.

JOHN G. McNAB.  
NILO V. HAKALA.  
JOHN P. McDERMOTT.

#### REFERENCES CITED

The following references are of record in the file of this patent:

#### UNITED STATES PATENTS

| Number    | Name     | Date          |
|-----------|----------|---------------|
| 2,261,047 | Assiff   | Oct. 4, 1941  |
| 2,364,154 | Denison  | Apr. 11, 1944 |
| 2,364,283 | Freuler  | Dec. 5, 1944  |
| 2,378,820 | Amott    | June 19, 1945 |
| 2,389,527 | McCleary | Nov. 20, 1945 |
| 2,420,893 | McNab    | May 20, 1947  |